

June 14, 1960      H. B. SNYDER ET AL      2,940,838

Agar solution containing  
high conc. of Acid +  
+ Chloride  
+ Nitrate  
+ Ferric ion  
+ wetting agent  
+ ammonium chlorostannate or mixt. of  $\text{K}_3\text{FeCl}_6$  + stannous chloride

CHEMICAL MILLING

Filed Aug. 19, 1957

annealed Steel

FIG. 1



FIG. 5



FIG. 2



FIG. 6



FIG. 3



FIG. 7



FIG. 8



FIG. 4



Ludwig M. Rosenberg  
Herman B. Snyder  
BY  
T W Secrest  
ATTORNEY

1

2,940,838

## CHEMICAL MILLING

Herman Ben Snyder and Ludwig M. Rosenberg, Seattle, Wash., assignors to Boeing Airplane Company, a corporation of Delaware

Filed Aug. 19, 1957, Ser. No. 678,882

8 Claims. (Cl. 41—42)

This discovery relates to the chemical milling of metal in an acid medium and, more particularly, to the chemical milling of age hardened, precipitation hardened and other heat treatable stainless steels in all their solid phases in an acid medium.

Prior to specifically discussing chemical milling we wish to point out the manner in which it distinguishes from pickling, brightening, decorative design and surface increase. Chemical milling may be considered to be controlled corrosion or controlled metal removal to form sculptured metal configurations. In chemical milling a relatively large percentage of the metal may be rapidly removed so as to leave a minor amount of the original metal in a new configuration. As contrasted with this is pickling or scale removal whereby as much as possible of the oxide and other coating of the metal are removed but as small amount as possible of the metal is removed. In other words in pickling only the surface coating of the metal is removed. In brightening or surface polishing a minimum amount of the metal is removed to form a reflective surface as the scale has been previously removed. Decorative designs are of a shallow depth with approximately five mils of surface removed by chemical action. In decorative design part of the surface is masked and the design is inscribed through the masked coating. Next, a chemical solution is applied to the masked material and allowed to react with the metal to form the design. An example of decorative design is silverware. In surface increase the object is to form a roughened surface. In order to specifically increase the surface area the same is purposely pitted by chemical action. This is done to make the surface rough enough for bonding purposes such as a metal to metal bond, a base for paint and the manufacture of condenser plates to name a few of the uses.

The mechanical milling of metal is well-known and extensively used throughout the metal working industry. Even though mechanical milling is extensively used it inherently has certain limitations. One of these limitations is the expensive capital investment for milling machines. Such a machine, capable of making large, complicated configurations, may cost in the hundreds of thousands of dollars. In addition to the capital investment it is necessary to have skilled workmen operating these machines in order to do a creditable job on the milling of metal. Also, because of cost and manhour requirements this type of milling is limited to certain configurations, namely, those configurations which are of a more simple or open design. However, by the skillful use of welding it is possible to build these limited configurations into an intricate design. Because of the nature of the weld and the inherent weakness therein it is not always advisable to build these limited basic configurations into an intricate design as the weld might rupture or the added weight become excessive. Furthermore, with mechanical milling there usually results a relatively rough surface. Because of excessive cost the tolerance, in a

2

recessed area, is not a close one but must be a rather large one such as in the hundreds of an inch. Also, on some of the newer metals it is impractical, because of cost due to equipment and to the time of milling involved, to mechanically mill the surfaces as the metal is extremely tough and resistant to mechanical cutting and/or rapid abrasion. For example, only casting and rough grinding can be employed with certain metals.

In recent years, as a supplement to mechanical milling, there has developed chemical milling. One of the first patents to be issued for chemical milling and the like is the patent to Wilson et al., United States Patent Number 2,684,291. Wilson et al. describe the embossing of steel with an acid medium. Basically, this patent presents the method of taking flat stock, masking certain predetermined areas or portions of this stock with an acid resistant covering, and etching the masked stock with the acidic solution. The acid solution eats away or corrodes away the unmasked areas to form the desired design. Naturally, it is possible to remove the stock from the acid solution, remove the masking cover, add new masking cover, and insert the stock again in the solution. By such means it is possible to form intricate designs in metal. With our discovery for the use of a strong acid solution in chemical milling we find it possible to realize a more rapid action than Wilson et al. realize with a weak acid solution; and to mill steel into predetermined designs and configurations while Wilson et al. are restricted to only surface change. Also, our strong acid milling solution makes it possible to work with equal ease on martensitic steels be they age hardened, precipitation hardened, or heat treated stainless steels.

To further illustrate some of the advantages of chemical milling it is possible to achieve the same output by chemical milling with a lower capital investment than for an equal output with mechanical milling. Also, in chemical milling the application of masking material to the part to be formed requires semi-skilled labor as contrasted with the requirement of skilled labor for mechanical milling. And, more intricate configurations can be formed more rapidly by chemical milling as the metal to be milled can be immersed in the reactant solution so that all parts of the metal can be acted upon simultaneously. In a specific illustration as applied to the manufacture of airplanes it is possible to reduce the weight of certain members of the airplane, as an example, stainless steel sheet stock may come in a thickness of 0.093 inch; however, from a design standpoint a thickness of 0.086 inch may be adequate. The original stock would not be reduced from the thickness of 0.093 inch to the thickness of 0.086 inch by mechanical milling as the cost would be too great, especially for heat treated stock. However, it is possible by chemical milling to immerse the stock in a chemical reactant solution and reduce it to the thickness desired with ease and economy. In large airplanes this reduction in thickness may mean a considerable saving in the weight of the air frame. More particularly, for every excess pound carried by the airplane there may be required from five to ten pounds of additional gross air frame weight. Therefore, if in the larger airplanes a thousand pounds of unneeded material can be saved the air frame weight can be reduced by approximately 5,000 pounds to 10,000 pounds.

In another manner the configuration of a chemically milled metal can be more economically achieved than by mechanical means. For example, in the case of a waffle pattern, the necessary chemical milling can be relatively easily performed as the masking materials can be placed over the metal and the metal not protected by this masking material can be chemically eaten away or chemi-

cally corroded. In a like manner an object can be tapered by removing the same slowly from the chemical milling solution. Also, an object having a large number of irregularly placed recessed areas can be readily manufactured by chemical milling while the preparation of a similar object by mechanical means would be time-consuming and difficult to prepare.

With this in mind it is an object of this discovery to provide a method for the chemical milling of metal, examples being intricate configurations, taper, and waffle pattern.

A further object is the provision of a method for the chemical milling of a metal and, particularly, for the chemical milling of age hardened, precipitation hardened and other heat treatable stainless steels in all their solid phases.

A further object is to provide a method for the chemical milling at a relatively uniform and controllable rate.

An additional object is to provide a solution for the chemical milling of metal and which solution can be controlled by standard methods of chemical analysis.

Another important object is the provision of a process for the chemical milling of metal and which process provides satisfactory surfaces having well defined edges at better than standard machine tolerances.

A still further object is the provision of a process for chemical milling resulting in satisfactory structural and mechanical properties of the milled metal.

A still further and important object is to provide for the chemical milling and which chemical milling results in a satisfactory smooth surface.

Another object is a provision of a process for chemical milling and which process produces a minimum of smut.

A further object is the provision of a process for chemical milling which is less expensive than mechanical milling and makes it possible to produce more intricate configurations than mechanical milling.

In the drawings:

Figure 1 is a plan view of a curved structural member illustrating two rectangular-shaped recesses in the open surface thereof.

Fig. 2 is a longitudinal vertical cross-sectional view taken on line 2-2 of Fig. 1 and shows the recesses in the curved member.

Fig. 3 is a view of a mask which is placed over the non-milled structural member in Fig. 1 and protects the upper surface of said structural member, except for the two rectangular shaped openings therein, from being attacked by the milling solution.

Fig. 4 is a longitudinal vertical cross sectional view of this curved raw material from which the structural member is prepared and illustrates this raw material as being covered with a protective masking coating except where the rectangular shaped recesses are to be formed.

Fig. 5, on an enlarged scale, shows the formation of a recess in metal with the aid of a masking material covering part of the metal.

Fig. 6 is an end elevation view of a curved structural member prior to chemical milling.

Fig. 7 is an end elevation view of the member in Figure 6 after being chemically milled to form a section for use in fabricating a fuel tank, and is taken on line 7-7 of Figure 8; and,

Fig. 8 is a plan view looking down on the chemically milled section of Figure 7.

In our chemical milling solution we provide an aqueous solution having a high concentration of acid, a chloride, a nitrate, a ferric ion, a moderator such as boric acid, oxalic acid or acetic acid, a wetting agent such as the sulfonic acid of an alkyl aryl compound, and ammonium chlorostannate or a mixture of stannic chloride and ammonium chloride. Each of these components plays a role in the chemical milling. Also, these components must be so balanced in their reaction with the components of the subject steels that the same is evenly cor-

roded by the chemical milling solution, i.e., all of the alloying elements of the steel are etched at the same rate as the iron or the base material of the steel. The hydrochloric acid appears to play a very active role in the chemical milling process. Also, the combination of the hydrochloric acid and the nitric acid appears to result in the aqua regia effect and plays an active role in the chemical milling. The addition of ferric chloride to hydrochloric acid and nitric acid speeds up or increases the corrosion rate.

10 This is especially so in regard to the corrosion of the iron in the steel. However, the ferric chloride, hydrochloric acid and nitric acid apparently react with the iron in the steel more quickly than they react with the alloying elements such as silicon, nickel and

15 molybdenum. Therefore, to increase the reaction rate of the composition with these alloying elements there is added ammonium chlorostannate or a mixture of stannic chloride and ammonium chloride. The addition of ammonium chlorostannate or the ammonium chloride and 20 stannic chloride mixture makes it possible for the milling solution to substantially uniformly corrode the martensitic steel. Therefore, both the base material, iron, and the alloying elements such as silicon, nickel and molybdenum are evenly eaten or corroded away. The moderator or buffer, having an ionization constant in the range of  $10^{-4}$   $10^{-6}$  with respect to the primary ionization constant of the hydrogen ion, appears to play the role of prolonging the active life of the milling solution. More 25 particularly, in a solution not having a moderator present the milling rate decreases almost immediately and continues to decrease at a substantially uniform rate throughout the life of the chemical milling solution. As is readily appreciated, with this decrease in the chemical milling rate the controlling of the milling or corrosion 30 of the metal being reacted upon is difficult. Also, there is an economical loss in the prolonging of the period of time the metal is in the solution as the milling bath is not being advantageously employed. However, with the incorporation of the moderator the reaction 35 proceeds at the same uniform rate for a relatively long period of time. Again, it is seen that with the reaction at a relatively uniform rate for a long period of time that it is possible to more readily control the milling of the metal thereby realizing a more desirable product as well 40 as being economically feasible to mill the metal. In regard to the wetting agent, such as an alkyl aryl sulfonate, i.e., dodecyl benzene sulfonate, this material makes it possible to achieve a better surface. The wetting agent probably functions by reducing the surface tension so as 45 to allow the gases produced by the action of the solution on the metal to more readily escape from the surface and therefore to permit a more uniform concentration of milling solution to react with the surface of the metal. It is realized that if the gases do not readily escape then 50 that portion of the metal covered by them will not be reacted upon the same as that portion not covered by the gas bubbles and therefore there would result an uneven or a less smooth surface.

In the milling solutions we prepared the nitrate was 55 added as hydrogen nitrate or nitric acid, the chloride as hydrogen chloride or hydrochloric acid, the acetate as hydrogen acetate or acetic acid, the citrate as hydrogen citrate or citric acid, the borate as hydrogen borate or boric acid, and the oxalate as oxalic acid or hydrogen oxalate.

In the milling process there are a number of factors determining the milling rate. Some of these factors are temperature, concentration of components, heat transfer, evaporation, agitation, volume of milling solution to surface area of metal, and so forth. Briefly, it is readily realized that the role of the temperature is very important. Generally speaking a ten degree rise in temperature, on the Kelvin scale, indicates a doubling in the reaction rate. Therefore, it is possible to achieve with a 60 relatively dilute or weak milling solution a milling rate

at a higher temperature equal to the milling rate of a more concentrated solution at a lower temperature. Also, it is apparent that the concentration of the reactant plays a very important and vital rôle in the chemical milling. In conjunction with the temperature effect it is possible by the use of a concentrated milling solution to achieve at a lower temperature the reaction rate equal to that of a relatively dilute solution at a higher temperature. This is of importance in the fact that a control of the milling can be obtained by control of the temperature. Heat transfer is of utmost importance as good heat transfer precludes the possibility of a local buildup of temperature and also is essential for the proper control of the milling rate. The local buildup of temperature means that in that particular area the reaction rate will be higher and more metal will be removed or corroded away. This uneven removal of the metal can result in uneven surfaces, pitting and tapering. Evaporation is of importance in that the evaporation of a vital component, viz., such as a chloride, means that the reaction rate will change in the life of the milling solution and the uniformity of the reaction rate cannot be as closely controlled as if evaporation had not taken place. Of great importance in the chemical milling of metal is the agitation of the solution. A well agitated solution gives more uniform results than one which is not agitated. This agitation may be in the form of mechanical agitation whereby the metal undergoing the milling action is vibrated or shaken back and forth in the milling bath. Another form of agitation may be that of the milling solution itself whereby it is agitated by gas bubbling through it. And, a still further and desirable form is that of ultrasonic vibration whereby high-frequency ultrasonic agitation is applied to the solution or to the metal undergoing reaction so as to break up any localized variations in the solution concentration. This also serves to avoid gas accumulation on the metal surface. Furthermore, the volume of the reacting chemical milling solution in proportion to the surface area of the material undergoing reaction can be of considerable importance. If the volume to surface ratio is rather low it is possible that the reactive components available at the milling surface will be rapidly exhausted and therefore there will be an uneven reaction rate and possibly an uneven removal of the metal affecting the quality of the finished product. Therefore, a large ratio of volume to surface area will give a more constant reaction rate and thus permit closer tolerances on the finished product.

To more particularly illustrate our discovery and especially the effects of the variation of the concentration of components and also the effect of the variation of the temperature we herewith present specific detailed examples. These examples are to be taken for illustrative purposes only and are not to be taken as limitations on the invention. In these examples the specifically enumerated components were utilized. More particularly, concen-

tated nitric acid of a specific gravity of approximately 1.42 and of a concentration of 68-70%; hydrochloric acid of a specific gravity of approximately 1.24 and a concentration of 38%; hydrofluoric acid of a specific gravity of 1.19 and 60% by weight; glacial acetic acid of a specific gravity of 1.055. Also, there were prepared a citric acid solution, an oxalic acid solution, and a boric acid solution. These three solutions were prepared by heating water to its boiling point and adding an excess of citric acid to one, boric acid to another, and oxalic acid to the other. The solutions were allowed to cool to room temperature and the supernatant liquid decanted from the precipitate. Examples of precipitation hardened, martensitic stainless and ferritic stainless steels are as follows: precipitation hardened, 17-7PH and 17-4PH comprising iron, carbon, silicon, manganese, chromium, nickel and copper; martensitic stainless steels are types 410, 420 and 440-A comprising in the main carbon, silicon, manganese and chromium. Other examples are types 414 S.S., 416 S.S., 440-B S.S., 440-C S.S., 440-F S.S., 431 S.S., 436 S.S., and 430 S.S. Other examples of martensitic steels are the SAE 4000 series such as 4130 and 4340.

Turning now to the tables and specific examples and embodiments of the invention it is to be realized that these examples are by way of illustration and teaching and are not meant to be limitations on the invention. In the main, these examples were run in a series of four or five. The concentration of the components was varied to determine the influence of the different components on the reaction rate. In order to arrive at reaction rates for average temperature it was decided that the base temperature should be in the range of 150-155° F. In some instances the temperature of the reaction solution was approximately 140° F. In other instances it was in the range of 160-170° F. And, in one or two cases it was about 200° F. If the temperature were approximately 140° F. the reaction rate was increased by about 25% to convert it to the range of about 150-155° F. Likewise, if the temperature were in the range of 160-175° F. the milling rate was decreased about 25% to bring it in the 150-155° F. range. It is to be appreciated that this is an approximation. In the tables the milling rate for the indicated temperature is given and the milling rate for the base temperature range is given in parentheses. The metals milled by the various solutions were AM350 and 17-7PH. The smoothness of the milled metal is expressed in "root mean square" terms, R.M.S., and the unit of measurement is micro inches of amplitude of surface variation.

In Table I there are presented four different solutions and the results of milling with these solutions. These solutions basically comprised water, hydrochloric acid and ferric chloride. In solution D there was also nitric acid. In this table the hydrochloric and nitric acids are expressed in terms of normality and the ferric chloride is expressed in molarity. These solutions were used to

Table I

| Variables                  | A                   |       | B                   |       | C                   |       | D                                                     |       |
|----------------------------|---------------------|-------|---------------------|-------|---------------------|-------|-------------------------------------------------------|-------|
|                            | Wt. Per. cent       | N     | Wt. Per. cent       | N     | Wt. Per. cent       | N     | Wt. Percent                                           | N     |
| HCl (38%)                  | 12.1                | 1.45  | 19.8                | 2.58  | 18.5                | 2.58  | 18.8                                                  | 2.48  |
| FeCl <sub>3</sub> (M)      | 9.8                 | 0.60  | 16.0                | 3.7   | 22.3                | 1.85  | 15.2                                                  | 1.23  |
| HNO <sub>3</sub> (68-70%)  |                     |       |                     |       |                     |       | 5.4                                                   | 1.79  |
| H <sub>2</sub> O           | 78.2                | ----- | 64.2                | ----- | 59.5                | ----- | 60.7                                                  | 0.79  |
|                            | 100.1               | ----- | 100.0               | ----- | 100.3               | ----- | 100.1                                                 | ----- |
| Metal                      | AM350               | ----- | AM350               | ----- | AM350               | ----- | AM350; 17-7PH                                         | ----- |
| Temperature, ° F.          | 140                 | ----- | 140                 | ----- | 140                 | ----- | 140                                                   | ----- |
| Milling Rate (Inches/min.) | 0.00004             | ----- | AM350-0.0000        | ----- | 0.0002              | ----- | 0.0006 (AM350)                                        | ----- |
|                            | (150° F., 0.00005.) | ----- | (150° F., 0.00013.) | ----- | (150° F., 0.00025.) | ----- | 0.00033 (17-7PH)                                      | ----- |
| R.M.S.                     |                     |       | 80-100              | ----- | 100-120             | ----- | (AM350, 150° F., 0.00075); (17-7PH, 150° F., 0.00044) | 45-50 |

mill AM350 at approximately 140° F. Comparison of solutions A, B and C shows that C milled faster than B which in turn milled faster than A. More particularly, C milled at about 0.0002 inch per minute as compared with B at 0.0001 and A at 0.00004 inch per minute. The concentration of the ferric chloride was increased from A through C. And, the concentration of the hydrochloric acid in both C and B was approximately 50% greater than in A. Turning now to solution D it is seen that the addition of the nitric acid considerably increased the reaction rate. Solution D may be considered to be very similar to solution B with the replacement of some of the water with nitric acid. The milling rate of D was about 0.0006 inch per minute as compared with approximately 0.0001 inch per minute for B. This increase in the reaction rate may be considered to be partially due to the increased total acid concentration in D. In summary, it may be stated that an increase in the concen-

solutions the concentrations of all the components were in the same range, varying from about 2.35 to about 3.36 normal for the hydrochloric acid, from about 0.69 to about 0.75 normal for the nitric acid, and from about 1.61 to approximately 2.3 molar for the ferric chloride. From this it is possible to state that a moderate variation in the concentration of the components does not appreciably affect the milling rates of the solutions. However, turning to solution D it is seen that the concentration of the nitric acid was increased appreciably to about 1.44 normal. The milling rate for this solution increased to about 0.0005 inch per minute or about 60%. Again, it is seen that an increase in the concentration of the nitric acid within reasonable limits, appreciably increases the milling rate. An alkyl aryl sulfonate was employed to assist in the reaction. More particularly, to permit greater penetration of solution to the surface of the metal.

Table II

| Variables                  | A                              |      | B                             |      | C                             |      | D                            |      |
|----------------------------|--------------------------------|------|-------------------------------|------|-------------------------------|------|------------------------------|------|
|                            | Wt. Percent                    | N    | Wt. Percent                   | N    | Wt. Percent                   | N    | Wt. Percent                  | N    |
| HCl (38%)                  | 17.5                           | 2.46 | 16.3                          | 2.46 | 24.1                          | 3.36 | 16.7                         | 2.35 |
| FeCl <sub>3</sub> (M)      | 22.2                           | 1.7  | 26.4                          | 2.3  | 19.4                          | 1.61 | 20.2                         | 1.68 |
| HNO <sub>3</sub> (68-70%)  | 5.0                            | 0.75 | 4.7                           | 0.75 | 4.6                           | 0.69 | 9.5                          | 1.44 |
| H <sub>2</sub> O           | 65.6                           |      | 62.6                          |      | 51.6                          |      | 53.6                         |      |
| Alkyl Aryl Sulfonate       | .1                             |      | .1                            |      | .1                            |      | .1                           |      |
|                            | 100.4                          |      | 100.1                         |      | 99.8                          |      | 100.1                        |      |
| Metal                      | AM350                          |      | AM350                         |      | AM350                         |      | AM350                        |      |
| Temperature, ° F.          | 140                            |      | 140                           |      | 140                           |      | 140                          |      |
| Milling Rate (inches/min.) | (0.0003)                       |      | (0.0003)                      |      | (0.0003)                      |      | (0.0005)                     |      |
|                            | (150° F., 0.000375, 0.000375.) |      | (150° F., 0.00045, 0.000375.) |      | (150° F., 0.00039, 0.000375.) |      | (150° F., 0.00062, 0.00062.) |      |
| R.M.S.                     | 70, 70                         |      | 90, 80                        |      | 60, 40                        |      | 70                           |      |

tration of the ferric ion increases the milling rate. Also, an increase in the total acid concentration increases the milling rate. As a sidelight, solution D was used to mill 17-7PH steel as well as AM350. The milling rate of 17-7PH steel was approximately 0.00035 inch per minute as compared with 0.0006 inch per minute for AM350.

Turning now to Table II another series of solutions was prepared comprising water, ferric chloride, hydrochloric acid and nitric acid. The concentrations of the components in these solutions were varied to bring forth the effects of the components on the milling rate. In this table the concentration of hydrochloric and nitric acids is indicated by normality while the concentration of the ferric chloride is expressed by molarity. A comparison of the milling rates of solutions A, B and C on AM350 at about 140° F. shows that they were substantially the same, i.e., about 0.0003 inch per minute. In these three

45 turning now to Table III another series of milling solutions was prepared. In this series the concentration of the nitric acid was varied over a wide range. Again the components were water, ferric chloride, hydrochloric acid and nitric acid. The hydrochloric and nitric acids were expressed in terms of normality and the ferric chloride in terms of molarity. The metal milled was AM350 and at a temperature of about 140° F. In this series of solutions solution A was solution D of Table I. The concentrations of the hydrochloric acid and the ferric chloride were maintained in about the same range, i.e., the hydrochloric acid varied from about 1.98 normal to about 2.35 normal and the ferric chloride varied from about 4.42 to 1.68 molar. However, the concentration of the 50 nitric acid was increased from 1.44 normal in solution A to 3.64 normal in solution E. The milling rate of solution A was the lowest, 0.0005 inch per minute. In solu-

Table III

| Variables                  | A                  |      | B                  |      | C                  |      | D                  |      | E                  |      |
|----------------------------|--------------------|------|--------------------|------|--------------------|------|--------------------|------|--------------------|------|
|                            | Wt. Percent        | N    | Wt. Percent        | N    | Wt. Percent        | N    | Wt. Percent        | N    | Wt. Percent        | N    |
| HCl (38%)                  | 16.7               | 2.35 | 15.9               | 2.24 | 15.2               | 2.15 | 14.6               | 2.07 | 14.0               | 1.98 |
| FeCl <sub>3</sub> (M)      | 20.2               | 1.68 | 19.2               | 1.60 | 18.4               | 1.54 | 17.6               | 1.48 | 16.9               | 1.42 |
| HNO <sub>3</sub> (68-70%)  | 9.5                | 1.44 | 13.6               | 2.06 | 17.4               | 2.63 | 20.8               | 3.06 | 24.0               | 3.64 |
| Alkyl Aryl Sulfonate       | .1                 |      | .1                 |      | .1                 |      | .1                 |      | .1                 |      |
| H <sub>2</sub> O           | 53.6               |      | 51.1               |      | 48.9               |      | 46.9               |      | 44.9               |      |
|                            | 100.1              |      | 99.9               |      | 100.0              |      | 100.0              |      | 99.9               |      |
| Metal                      | AM350              |      | AM350              |      | AM350              |      | AM350              |      | AM350              |      |
| Temperature (° F.)         | 140                |      | 140                |      | 140                |      | 140                |      | 140                |      |
| Milling Rate (inches/min.) | 0.0005             |      | 0.00057            |      | 0.00082            |      | 0.00053            |      | 0.00066            |      |
|                            | (150° F., 0.00071) |      | (150° F., 0.00071) |      | (150° F., 0.00103) |      | (150° F., 0.00065) |      | (150° F., 0.00070) |      |
| R.M.S.                     | 70                 |      | 60                 |      | 65                 |      | 130                |      | 65                 |      |

tion B the milling rate was 0.00057 inch per minute, a slight increase over solution A. In solution C, with a concentration of nitric acid at 2.63 normal the milling rate was the highest for the series, 0.00082 inch per minute. With a further increase in the concentration of the nitric acid, see solutions D and E, the milling rate decreased to approximately that for solutions A and B. This indicates that the increase in the concentration of nitric acid is beneficial to a certain concentration and then it is of no further value and actually retards the re-

about 120-140° F. Solution A was the fundamental solution. Solution B was similar to solution A except that the concentration of the ferric chloride was increased approximately by one third. Solution C was similar to solution A except that there was added ferric nitrate so as to increase the concentration of the ferric salt. And, solution D was also similar to A except that there was added ferric sulfate to increase the concentration of the ferric salt. The milling rate of all of these solutions was in the same range, i.e., 0.0003 to 0.0006 inch per minute.

Table IV

| Variables                                           | A           |      | B             |      | C           |      | D           |      |
|-----------------------------------------------------|-------------|------|---------------|------|-------------|------|-------------|------|
|                                                     | Wt. Percent | N    | Wt. Percent   | N    | Wt. Percent | N    | Wt. Percent | N    |
| HCl (33%)                                           | 16.6        | 2.34 | 15.6          | 2.34 | 15.6        | 2.34 | 15.6        | 2.34 |
| FeCl <sub>3</sub> (M)                               | 20.2        | 1.65 | 25.2          | 2.24 | 18.9        | 1.65 | 18.9        | 1.65 |
| HNO <sub>3</sub> (68-70%)                           | 9.5         | 1.43 | 9.0           | 1.43 | 8.9         | 1.43 | 8.9         | 1.43 |
| Fe(NO <sub>3</sub> ) <sub>3</sub> (M)               |             |      |               |      | 6.3         | 1.24 |             |      |
| Fe <sub>2</sub> (SO <sub>4</sub> ) <sub>3</sub> (M) |             |      |               |      |             |      | 6.3         | 0.75 |
| H <sub>2</sub> O                                    | 53.6        |      | 50.3          |      | 50.3        |      | 50.3        |      |
|                                                     | 99.9        |      | 100.1         |      | 100.0       |      | 100.0       |      |
| Metal                                               | AM350       |      | AM350         |      | AM350       |      | AM350       |      |
| Temperature (° F.)                                  | 120-140     |      | 120-140       |      | 120-140     |      | 120-140     |      |
| Milling Rate (inches/min.)                          | 0.0005      |      | 0.0004-F      |      | 0.0006      |      | 0.0003      |      |
|                                                     |             |      | 0.0007        |      |             |      |             |      |
|                                                     |             |      | (160° F.)     |      | (150° F.,   |      | (150° F.,   |      |
|                                                     |             |      | (120-140° F., |      | 0.0006      |      | 0.00045     |      |
|                                                     |             |      | 0.00075)      |      | 160° F.,    |      |             |      |
|                                                     |             |      |               |      | 0.00052     |      |             |      |
| R.M.S.                                              | 90          |      | 55            |      |             |      |             |      |

action rate. More particularly, it may be surmised that too high a concentration of the nitric acid passivates the surface of the metal being milled. Possibly there is formed an oxide layer on the surface which acts as a membrane to decrease the flow of active components in the solution to the metal. Again, an alkyl aryl sulfonate such as the sodium salt of dodecyl benzene sulfonic acid was incorporated into the aqueous reaction solution. This salt appears to have decreased the surface tension of the solution so as to allow the same to penetrate to the surface of the metal for greater ease of reaction.

There was prepared another series of milling solutions, see Table IV, in which the concentration of the ferric salt was varied and in which different ferric salts were employed. The fundamental solution comprised water, ferric chloride, hydrochloric acid and nitric acid. This

In Table V there is illustrated another series of milling 35 solutions. Again, the fundamental solution comprised water, ferric chloride, hydrochloric and nitric acids. The concentrations of the hydrochloric and nitric acids are expressed in terms of normality and the concentration of the ferric chloride is in terms of molarity. These solutions 40 were employed to mill AM350 in the temperature range of about 160-170° F. Solution A was the fundamental solution. Solution B was similar to solution A but comprised about 3.2% by weight of acetic acid. 45 Solution C was similar to A except that it comprised about 3.2% by weight of glycerine. The milling rates of A and B were substantially the same, 0.0008 and 0.0007 inch per minute. The milling rate of solution C was considerably less than these two as it was 0.0002 inch 50 per minute.

Table V

| Variables                  | A           |      | B           |      | C           |      |
|----------------------------|-------------|------|-------------|------|-------------|------|
|                            | Wt. percent | N    | Wt. percent | N    | Wt. percent | N    |
| HCl (33%)                  | 15.6        | 2.35 | 15.1        | 2.22 | 15.1        | 2.22 |
| FeCl <sub>3</sub> (M)      | 25.2        | 2.24 | 24.4        | 2.13 | 24.4        | 2.13 |
| HNO <sub>3</sub> (68-70%)  | 9.0         | 1.43 | 8.6         | 1.38 | 8.6         | 1.38 |
| H <sub>2</sub> O           | 50.4        |      | 48.6        |      | 48.6        |      |
| Acetic acid                |             |      | 3.2         |      |             |      |
| Glycerine                  |             |      |             |      | 3.2         |      |
|                            | 100.2       |      | 99.9        |      | 99.9        |      |
| Metal                      | AM350       |      | AM350       |      | AM350       |      |
| Temperature, ° F.          | 160-170     |      | 160-170     |      | 160-170     |      |
| Milling Rate (inches/min.) | 0.0008      |      | 0.0007      |      | 0.0002      |      |
|                            | (150° F.,   |      | (150° F.,   |      | (150° F.,   |      |
|                            | 0.0006)     |      | 0.00053     |      | 0.00015     |      |
| R.M.S.                     | 65          |      | 65          |      | 100         |      |

solution was varied by adding ferric chloride, ferric nitrate or ferric sulfate. In this table the concentrations of the hydrochloric and nitric acids are expressed in terms of normality and the concentrations of the ferric salts are expressed in terms of molarity. These solutions were employed to mill AM350 at a temperature in the range of 70

Another series of milling solutions was prepared comprising water, ferric chloride, hydrochloric and nitric acids. The results of this series are presented in Table VI. To this fundamental solution there was added ammonium chloride, stannic chloride and ammonium chlorostannate. In this table the ferric chloride, ammonium

chloride, stannic chloride and ammonium chlorostannate were expressed in terms of molarity and the nitric acid and hydrochloric acid in terms of normality. These solutions were employed to mill AM350 in the temperature range of about 160-170° F. The fundamental or control solution was solution A. The milling rate of this solution was about 0.0005 inch per minute. Solution B was similar to A except that there was added ammonium chloride. The milling rate of solution B was 0.0008 inch per minute, an increase of about 35% over the milling rate of A. Solution C was also similar to A

5

10

of E was slightly lower than D, due to the lower milling temperature. Solution E milled AM350 at 0.0011 inch per minute, faster than it milled 17-7PH, 0.00025 inch per minute. In summary, the addition of ammonium chloride to the fundamental solution increased the reaction rate. The addition of stannic chloride increased the reaction rate almost three fold over that of the fundamental solution. And, the addition of both ammonium chloride and stannic chloride increased the reaction over that of the fundamental solution and also gave a smoother surface than the control solution gave.

Table VI

| Variables                                 | A                       |                       | B                      |                       | C                     |                       | D                     |                       | E                     |                       |
|-------------------------------------------|-------------------------|-----------------------|------------------------|-----------------------|-----------------------|-----------------------|-----------------------|-----------------------|-----------------------|-----------------------|
|                                           | Wt. Percent             | N                     | Wt. Percent            | N                     | Wt. Percent           | N                     | Wt. Percent           | N                     | Wt. Percent           | N                     |
| HCl(38%)                                  | 15.6                    | 2.34                  | 14.7                   | 2.34                  | 14.7                  | 2.34                  | 14.7                  | 2.34                  | 14.7                  | 2.34                  |
| FeCl <sub>3</sub> (M)                     | 25.2                    | 2.23                  | 23.6                   | 2.23                  | 23.6                  | 2.23                  | 23.6                  | 2.23                  | 23.6                  | 2.23                  |
| HNO <sub>3</sub> (68-70%)                 | 8.9                     | 1.44                  | 8.4                    | 1.44                  | 8.4                   | 1.44                  | 8.4                   | 1.44                  | 8.4                   | 1.44                  |
| H <sub>2</sub> O                          | 50.3                    | -----                 | 47.3                   | -----                 | 47.3                  | -----                 | 47.3                  | -----                 | 47.3                  | -----                 |
| NH <sub>4</sub> Cl(M)                     | -----                   | 5.9                   | 1.7                    | -----                 | 5.9                   | 0.4                   | 1.5                   | 0.4                   | 1.5                   | 0.4                   |
| SnCl <sub>4</sub> (M)                     | -----                   | -----                 | -----                  | -----                 | -----                 | -----                 | (NH <sub>4</sub> Cl)  | 4.4                   | (NH <sub>4</sub> Cl)  | 4.4                   |
| SnCl <sub>4</sub> ·2NH <sub>4</sub> Cl(M) | -----                   | -----                 | -----                  | -----                 | -----                 | -----                 | (SnCl <sub>4</sub> )  | 0.25                  | (SnCl <sub>4</sub> )  | 0.25                  |
|                                           | 100.0                   | 99.9                  |                        | 99.9                  |                       | 99.9                  |                       | 99.9                  |                       | 99.9                  |
| Metal                                     | AM350                   | AM350                 | AM350                  | AM350                 | AM350                 | AM350                 | AM350                 | AM350                 | AM350                 | AM350                 |
| Temperature (° F.)                        | 160-170                 | 160-170               | 160-170                | 160-170               | 160-170               | 160-170               | 160-170               | 160-170               | 160-170               | 160-170               |
| Milling Rate (inches/min.)                | 0.0005                  | 0.0008                | 0.0011                 | 0.0014                | 0.0016                | 0.0018                | 0.0020                | 0.0022                | 0.0025                | 0.0028                |
|                                           | (160° F.,<br>0.000375.) | (160° F.,<br>0.0006.) | (160° F.,<br>0.00105.) | (160° F.,<br>0.0014.) | (160° F.,<br>0.0018.) | (160° F.,<br>0.0022.) | (160° F.,<br>0.0025.) | (160° F.,<br>0.0028.) | (160° F.,<br>0.0032.) | (160° F.,<br>0.0035.) |
| R.M.S.                                    | 60.                     | 45.                   | 55.                    | 50.                   | 50.                   | 50.                   | 50.                   | 50.                   | 50.                   | 50.                   |

except that there was incorporated stannic chloride. The milling rate for C, 0.0014 inch per minute, was almost three times the milling rate of A, 0.0005 inch per minute. As is seen, the addition of the stannic chloride considerably increased the milling rate. Solution D combined all the components so that it was similar to A but with the addition of ammonium chloride and stannic chloride. The ammonium chloride and stannic chloride can be considered to be ammonium chlorostannate. The milling rate of D was comparable to that of C, 0.0013 inch per minute. In the table the ammonium chloride and the stannic chloride in solution D were expressed as being separate but it is to be realized that in actuality they were in the form of ammonium chlorostannate. Solution E was substantially the same as solution D. However, the milling temperature of E was approximately 15° lower than for D. Also, solution E was used to mill both AM350 and 17-7PH steels. The milling rate

35 In Table VII there is presented another set of milling solutions having water, ferric chloride, nitric acid and hydrochloric acid. This fundamental solution was varied by the addition of boric acid, phosphoric acid or oxalic acid. In this table the hydrochloric and nitric acids are 40 expressed in terms of normality and the ferric chloride, boric acid, phosphoric and oxalic acids are expressed in terms of molarity. These solutions were used to mill AM350 in the temperature range of about 160-170° F. Solution A was the control solution and milled at the 45 rate of about 0.0007 inch per minute. Solution B was similar to A except that there was added boric acid and it milled at the rate of about 0.0008 inch per minute. Solution C was similar to A except that it contained phosphoric acid and milled at the rate of approximately 50 0.0007 inch per minute. Solution D was similar to A but contained oxalic acid and milled at the rate of about 0.0006 inch per minute. Also, solution D was employed

Table VII

| Variables                  | A                      |                       | B                     |                       | C                     |                       | D                     |                       |
|----------------------------|------------------------|-----------------------|-----------------------|-----------------------|-----------------------|-----------------------|-----------------------|-----------------------|
|                            | Wt. Percent            | N                     | Wt. Percent           | N                     | Wt. Percent           | N                     | Wt. Percent           | N                     |
| HCl (38%)                  | 15.6                   | 2.34                  | 14.7                  | 2.34                  | 14.7                  | 2.34                  | 14.7                  | 2.34                  |
| FeCl <sub>3</sub> (M)      | 25.2                   | 2.23                  | 23.6                  | 2.23                  | 23.6                  | 2.23                  | 23.6                  | 2.23                  |
| HNO <sub>3</sub> (68-70%)  | 8.9                    | 1.44                  | 8.4                   | 1.44                  | 8.4                   | 1.44                  | 8.4                   | 1.44                  |
| H <sub>2</sub> O           | 50.3                   | -----                 | 47.3                  | -----                 | 47.3                  | -----                 | 47.3                  | -----                 |
| Boric Acid (M)             | -----                  | 5.9                   | 1.47                  | -----                 | 5.9                   | 1.47                  | 5.9                   | 1.47                  |
| Phosphoric Acid (M)        | -----                  | -----                 | -----                 | -----                 | -----                 | -----                 | 5.9                   | 1.0                   |
| Oxalic Acid (M)            | -----                  | -----                 | -----                 | -----                 | -----                 | -----                 | -----                 | -----                 |
|                            | 100.0                  | 99.9                  |                       | 99.9                  |                       | 99.9                  |                       | 99.9                  |
| Metal                      | AM350                  | AM350                 | AM350                 | AM350                 | AM350                 | AM350                 | AM350                 | AM350                 |
| Temperature, ° F.          | 160-170                | 160-170               | 160-170               | 160-170               | 160-170               | 160-170               | 160-170               | 160-170               |
| Milling Rate (inches/min.) | 0.0007                 | 0.0008                | 0.0009                | 0.0007                | 0.0008                | 0.0007                | 0.0006                | 0.0005                |
|                            | (160° F.,<br>0.00053.) | (160° F.,<br>0.0006.) | (160° F.,<br>0.0008.) | (160° F.,<br>0.0007.) | (160° F.,<br>0.0009.) | (160° F.,<br>0.0007.) | (160° F.,<br>0.0006.) | (160° F.,<br>0.0005.) |
| R.M.S.                     | 60.                    | 50.                   | 50.                   | 50.                   | 50.                   | 50.                   | 50.                   | 50.                   |

to mill 17-7PH steel with a milling rate of about 0.0005 inch per minute.

Table VIII presents the summary of the results with two milling solutions. These solutions comprised water, nitric acid, citric acid, hydrochloric acid, hydrofluoric acid, acetic acid and disodium monohydrogen phosphate. Solution B differed from A in that B contained a ferric salt, ferric nitrate. In this table the ferric salt is expressed in terms of molarity and the concentration of the nitric acid, acetic acid, hydrochloric and hydrofluoric acids are expressed in terms of normality. These solutions were employed to mill 17-7PH steel at approximately room temperature. Solution A, without the benefit of the ferric salt, milled at the rate of 0.0001 inch per minute. Solution B, with the benefit of the ferric salt, milled at the rate of 0.0003 inch per minute. From these results it is possible to state that the addition of a ferric salt increases the milling rate of the solution on 17-7PH metal.

Table VIII

| Variables                                | A           |       | B           |       |
|------------------------------------------|-------------|-------|-------------|-------|
|                                          | Wt. Percent | N     | Wt. Percent | N     |
| HNO <sub>3</sub> (68-70%)                | 20.9        | 2.58  | 20.6        | 2.58  |
| Acetic Acid (glacial)                    | 2.3         | 0.4   | 2.3         | 0.4   |
| HCl (38%)                                | 9.2         | 1.06  | 9.0         | 1.06  |
| HF (60%)                                 | 13.1        | 4.37  | 13.0        | 4.37  |
| Citric Acid (sat'd)                      | 0.6         | ----- | 0.6         | ----- |
| Na <sub>2</sub> HPO <sub>4</sub> (sat'd) | 0.6         | ----- | 0.6         | ----- |
| H <sub>2</sub> O                         | 53.5        | ----- | 52.7        | ----- |
| Fe(NO <sub>3</sub> ) <sub>3</sub> (M)    | -----       | ----- | 1.8         | 0.07  |
|                                          | 100.2       | ----- | 100.6       | ----- |
| Metal                                    | 17-7PH      | ----- | 17-7PH      | ----- |
| Temperature, °F                          | Room        | ----- | Room        | ----- |
| Milling Rate (inches/min.)               | 0.0001      | ----- | 0.0003      | ----- |
| R.M.S.                                   | 80-100      | ----- | 190-250     | ----- |

Table IX presents the results of milling with two other milling solutions. These solutions comprised water, nitric acid, acetic acid, hydrochloric acid, hydrofluoric acid, hydrobromic acid, citric acid and disodium monohydrogen phosphate. In this table the concentrations of the ferric salt is expressed in terms of molarity and the concentrations of the nitric acid, acetic acid, hydrochloric acid, hydrofluoric acid and hydrobromic acid are in terms of normality. These solutions were used to mill 17-7PH steel at approximately room temperature. Solution B varied from solution A in that the former contained a ferric salt, ferric nitrate. Solution A, without the benefit of ferric salt, milled this steel at the rate of 0.0001 inch per minute. Solution B, with the benefit of the ferric salt, milled this metal at the rate of 0.00022 inch per minute. Again, it is possible to state that the addition of a ferric salt to a milling solution increases the milling rate on martensitic steel.

Table IX

| Variables                                | A           |       | B           |       |
|------------------------------------------|-------------|-------|-------------|-------|
|                                          | Wt. Percent | N     | Wt. Percent | N     |
| HNO <sub>3</sub> (68-70%)                | 19.8        | 2.48  | 19.5        | 2.48  |
| Acetic Acid (glacial)                    | 2.2         | 0.4   | 2.1         | 0.4   |
| HCl (38%)                                | 8.8         | 1.02  | 8.8         | 1.02  |
| HF (60%)                                 | 12.4        | 4.2   | 12.2        | 4.2   |
| HBr                                      | 5.1         | 0.3   | 5.0         | 0.3   |
| Citric Acid (Sat'd)                      | 0.5         | ----- | 0.5         | ----- |
| Na <sub>2</sub> HPO <sub>4</sub> (Sat'd) | 0.5         | ----- | 0.5         | ----- |
| H <sub>2</sub> O                         | 50.6        | ----- | 49.8        | ----- |
| Fe(NO <sub>3</sub> ) <sub>3</sub> (M)    | -----       | ----- | 1.7         | 0.7   |
|                                          | 99.9        | ----- | 99.8        | ----- |
| Metal                                    | 17-7PH      | ----- | 17-7PH      | ----- |
| Temperature, °F                          | Room        | ----- | Room        | ----- |
| Milling Rate (inches/min.)               | 0.0001      | ----- | 0.00022     | ----- |
| R.M.S.                                   | 150-220     | ----- | 180-230     | ----- |

Table X presents the summary of milling with two other milling solutions. These solutions comprised water, nitric acid, acetic acid, hydrofluoric acid, citric acid, and disodium monohydrogen phosphate. In this table the concentration of the ferric salt is expressed in terms of molarity and the concentrations of the nitric acid, acetic acid and hydrofluoric acid are in terms of normality. These solutions were employed to mill 17-7PH metal at approximately room temperature. Solution B differed from A in that the former comprised ferric nitrate while the latter did not. The milling rate of solution A, without benefit of the ferric salt, was 0.00002 inch per minute. The milling rate of solution B, with benefit of the ferric salt, was 0.00008 inch per minute. Again it is possible to state that the addition of a ferric salt to a milling solution increases the milling rate of the solution on martensitic steel.

Table X

| Variables                                | A           |       | B           |       |
|------------------------------------------|-------------|-------|-------------|-------|
|                                          | Wt. Percent | N     | Wt. Percent | N     |
| HNO <sub>3</sub> (68-70%)                | 23.0        | 2.82  | 22.6        | 2.82  |
| Acetic acid (glacial)                    | 2.5         | 0.5   | 2.5         | 0.5   |
| HF (60%)                                 | 14.5        | 4.75  | 14.2        | 4.75  |
| Citric Acid (Sat'd)                      | 0.6         | ----- | 0.6         | ----- |
| Na <sub>2</sub> HPO <sub>4</sub> (Sat'd) | 0.6         | ----- | 0.6         | ----- |
| H <sub>2</sub> O                         | 58.9        | ----- | 57.8        | ----- |
| Fe(NO <sub>3</sub> ) <sub>3</sub>        | 2.0         | 0.08  | -----       | ----- |
|                                          | 100.1       | ----- | 100.3       | ----- |
| Metal                                    | 17-7PH      | ----- | 17-7PH      | ----- |
| Temperature, °F                          | Room        | ----- | Room        | ----- |
| Milling Rate (inches/min.)               | 0.00002     | ----- | 0.00008     | ----- |
| R.M.S.                                   | 55-85       | ----- | 70-80       | ----- |

At this time it is proper to compare the results of the milling solutions in Tables VIII, IX and X. The milling solutions in Tables VIII and IX comprised hydrochloric acid. The milling solutions in Table X did not have the benefit of the hydrochloric acid. It is seen that the milling solution comprising hydrochloric acid milled at an increased rate over the milling solutions not having hydrochloric acid. More particularly, in Tables VIII and IX the milling solutions having hydrochloric acid but not having a ferric salt milled at the rate of 0.0001 inch per minute. A corresponding solution in Table X not having hydrochloric acid and not having the benefit of a ferric salt milled at the rate of 0.00002 inch per minute. In other words, the milling solution without benefit of hydrochloric acid milled at a rate of one-sixth of those solutions having the benefit of hydrochloric acid. Furthermore, for those milling solutions having both hydrochloric acid and the benefit of ferric ion the milling rate was greater than for the milling solutions not having either hydrochloric acid or ferric ion. Solution B in Table IX, having both hydrochloric acid and ferric ion, had a milling rate of 0.00022 inch per minute. Solution B in Table VIII, having both hydrochloric acid and ferric ion, had a milling rate of about 0.0003 inch per minute. Solution B in Table X, having neither hydrochloric acid nor ferric salt, had a milling rate of about 0.00008 inch per minute. It is seen that the milling rates of solutions B in Tables VIII and IX are at least ten times the milling rate of solution B in Table X. These two series of data illustrate the value of hydrochloric acid in a milling solution.

A further series of milling solution was prepared. This series comprised water, nitric acid, acetic acid, hydrofluoric acid, citric acid, disodium monohydrogen phosphate and ferric nitrate. In this table the nitric acid, hydrofluoric acid and acetic acid are expressed in terms of normality and the ferric salt in terms of molarity. These solutions were used to mill 17-7PH steel at various temperatures ranging from room temperature to about 200° F. The fundamental solution was A and

comprised water, nitric acid, acetic acid, hydrofluoric acid, citric acid, disodium monohydrogen phosphate and ferric chloride. This solution milled at the rate of 0.00014 inch per minute. To a solution such as A there was added ferric nitrate to form B. Solution B milled at the rate of 0.00033 inch per minute. The milling rate of B was over twice the rate of A. From this it is possible to state that the addition of ferric nitrate to a milling solution, or the increase of the ferric ion in the milling solution, increases the milling rate. To a solution such as C there was added powdered titanium to form C. Solution C milled 17-7PH steel at temperatures of 80° and 145° F. As the milling temperatures of A and B were room temperatures, it is not possible to compare the milling rate of C with these. However, it is seen that at 80° F. the milling rate was lower than for A and B and at 145° F. the milling rate was greater than for A and B. To a solution such as C there was added aluminum nitrate to form solution D. This solution milled at a temperature of 135° F. and the milling rate was 0.0011 inch per minute. It is seen that the addition of aluminum nitrate to the milling solution increased the milling rate. To a solution such as D there was added a powdered aluminum alloy, 75S, to make solution E. The milling temperature of this solution was 200° F. and the rate was 0.00026 inch per minute. These results are tabulated in Table XI.

to be chemically milled and is dipped or submerged in the milling solution for a predetermined time. With the passing of the time the milling solution eats away or corrodes away the metal so as to form the two recesses 11. It is to be noted that that portion of the metal covered by the protective neoprene film is not attacked and only that portion of the metal not covered by the protective film is corroded away. After the passage of a predetermined time and the recesses are of a sufficient depth and size the structural panel is removed from the milling solution. The adherent solution is washed away and the neoprene protective film stripped off the panel to produce that shown in Figure 1. Other teachings for the masking of metal may be found in United States Patents Numbers 2,739,047 to Sanz and 2,684,291 to Wilson et al.

In Figure 5 there is illustrated the action of the milling solution on the metal at the junction of the protective film and the metal. It is seen that milling solution 16 eats away metal 17 so as to undercut protective film 18. One of the particular advantages of the use of a wetting agent is to induce better contact between the milling solution and the metal. With a better contact or a lowering of the effective surface tension there is less possibility of gases collecting on the surface or near masked edges underneath the protective film. For this function there are a number of suitable wetting agents such as pine oil. One of the common wetting agents is an alkyl aryl sul-

Table XI

| Variables                                | A           |      | B           |      | C             |      | D            |      | E           |      |
|------------------------------------------|-------------|------|-------------|------|---------------|------|--------------|------|-------------|------|
|                                          | Wt. Percent | N    | Wt. Percent | N    | Wt. Percent   | N    | Wt. Percent  | N    | Wt. Percent | N    |
| HNO <sub>3</sub> (68-70%)                | 20.2        | 2.48 | 19.8        | 2.48 | 19.7          | 2.48 | 19.5         | 2.48 | 19.3        | 2.48 |
| Acetic acid (glacial)                    | 2.2         | 0.4  | 2.2         | 0.4  | 2.1           | 0.4  | 2.1          | 0.4  | 2.1         | 0.4  |
| HF (60%)                                 | 12.6        | 4.2  | 12.4        | 4.2  | 12.3          | 4.2  | 12.2         | 4.2  | 12.1        | 4.2  |
| Citric Acid (Sat'd)                      | 0.6         | —    | 0.6         | —    | 0.6           | —    | 0.5          | —    | 0.5         | —    |
| Na <sub>2</sub> HPO <sub>4</sub> (Sat'd) | 0.6         | —    | 0.6         | —    | 0.6           | —    | 0.5          | —    | 0.5         | —    |
| H <sub>2</sub> O                         | 62.1        | 61.0 | 60.6        | 60.0 | 60.6          | 60.0 | 59.4         | 59.4 | 59.4        | 59.4 |
| FeCl <sub>3</sub> (M)                    | 1.8         | 0.12 | 1.8         | 0.12 | 1.7           | 0.12 | 1.7          | 0.12 | 1.7         | 0.12 |
| Fe(NO <sub>3</sub> ) <sub>3</sub> (M)    | —           | —    | 1.8         | 0.07 | 1.7           | 0.07 | 1.7          | 0.07 | 1.7         | 0.07 |
| Ti                                       | —           | —    | —           | —    | 0.7           | —    | 0.7          | —    | 0.7         | —    |
| Al(NO <sub>3</sub> ) <sub>3</sub>        | —           | —    | —           | —    | —             | —    | —            | —    | —           | 0.8  |
| 75 S                                     | —           | —    | —           | —    | —             | —    | —            | —    | —           | —    |
| Metal                                    | 17-7PH      | —    | 17-7PH      | —    | 17-7PH        | —    | 17-7PH       | —    | 17-7PH      | —    |
| Temperature (° F.)                       | Room        | —    | Room        | —    | 80, 145       | —    | 235          | —    | 200         | —    |
| Milling Rate (inches/min.)               | 0.000144    | —    | 0.00033     | —    | { 80-0.00092  | —    | 0.0011       | —    | 0.00025     | —    |
| R.M.S.                                   | 90-110      | —    | 130-180     | —    | { 145-0.00076 | —    | { 80-100-130 | —    | 100-150     | —    |
|                                          |             |      |             |      | { 145-80-120  | —    |              |      | 90-130      | —    |

Having described our discovery and illustrated the same with reference to various compositions of matter for the use of chemical milling solution, reference is hereby made to the practical application of these solutions. Referring to the drawings, and especially Figure 1, it is seen that there is illustrated a structural panel 10 having two chemically milled recesses 11 therein. In Figure 2, a vertical cross-sectional view of Figure 1, it is seen that this structural panel is curved and that these two recesses are separated from each other by a rib 12. In the manufacture of this type of structural panel the material to be saved is covered by an adhering and strippable protective film or coating, there are numerous such coatings or films examples being neoprene, vinyl etch-proof film, and others. More particularly, for shallow milling there may be used various acid resistant paints. To pictorially illustrate the making of this structural panel reference is made to Figures 3 and 4. In Figure 3 there is illustrated a neoprene mask 13 having two recesses 14 therein. This neoprene film 13 is placed on the concave side of the structural panel 10 and on the edges and the convex side are attached other protective neoprene films. A cross-sectional view of the structural panel before chemical milling takes place is shown in Figure 4 whereby the panel is covered by the neoprene having the two cutouts 14 illustrated therein. This structural panel is now ready

50 fonate. Specific sulfonates which are useful are the sodium salts of dodecyl benzene sulfonic acid and pentadecyl benzene sulfonic acid.

Another instance where our solution is of value is in the chemical milling of components for aircraft. In Figure 6 is illustrated a curved structural plate having a thickness of 0.750 inch. This plate was transformed into a structural member, for use in a fuel tank, having a thickness of 0.100 inch. The finished product, see Figures 7 and 8, was prepared from the original structural plate by masking the two central portions so as to form the boss upon the corrosion of the surrounding metal. As is seen, one of these bosses is 0.500 inch in thickness and the other boss is 0.750 in thickness. Each of these is tapped. The outside perimeter of this section is formed into a thickness of 0.250 inch, approximately two and one-half times as thick as the main part of the section. The increased thickness of the perimeter is for added strength upon the welding of this section into the main part of the fuel tank. Normally such a section would be formed by fabrication using a welding technique. However, the welding process causes grain growth which in turn causes a weakening of the metal. With our method there is no grain growth.

70 The control for determining the degree of chemical milling may be carried out in a number of different man-

ners. One of these is to introduce a material of a predetermined thickness into the chemical milling solution along with the member to be chemically milled and to periodically weigh or measure this member. When this member has decreased a certain amount in weight or thickness it is possible to decide whether the structural member undergoing chemical milling has been corroded away sufficiently.

Returning now to the metals and the examples presented therein it is noticed that the smoothness of R.M.S. values are mainly in the range of approximately 50-125 R.M.S. This is of a special importance as this value represents a surface that is relatively smooth. In fact, the milled metal is often smoother than the metal when machine milled. In machine milling the average smoothness value is approximately 125 R.M.S. Of course, this value of 125 R.M.S. is subject to variation as with soft alloys it is possible to machine mill the metal somewhat smoother than 125 R.M.S., but with heat treated, work hardened and tempered alloys which may have a tough surface skin it is difficult to achieve a smoothness value of 125 R.M.S. on machine milling. However, with this chemical milling process it is possible to achieve a smoothness value which approaches that used for mirrors and reflective surfaces, and it is possible to achieve this smoothness on all types of alloys be they hard, heat treated, work hardened, or tempered.

The smoothness values were determined by a profilometer. The profilometer used possessed a diamond needle which rode on the surface of the metal and measured the profile of the surface in millionths of an inch in amplitude. These measurements are expressed in R.M.S. or root means square values. Such an instrument is commercially obtainable from Physicists Research Company, Ann Arbor, Michigan.

In this chemical milling process it is noticed that there is little if any smut. Smut is defined as that material which clings to the metal itself. Smut is usually an oxide of the alloy or chemical compounds of the alloy or unreacted finely divided alloying materials and is attracted to the bulk metal by electrochemical and electrostatic forces.

With our process in chemical milling it is possible to achieve tolerances in some usages which have not been obtainable in commercial practice before. These tolerances are in the range of approximately plus or minus 0.0005 inch, making it possible to achieve a high quality and/or a precision product. Also, in our process it has been observed that there is no intergranular corrosion due to the chemical action of the solutions. This success in not having intergranular corrosion makes it possible to achieve higher strength components for less weight of the component as compared with the presently machine milled and welded components.

Our process is also adaptable for a continuous method or a batch method. In the continuous process it is possible to contact the structural item to be made with the milling solution and to continuously recirculate the milling solution so as to maintain uniformity of solution in contact with all reacting surfaces. Chemical processing equipment, i.e., tanks, pipe fittings, valves, and pumps lined with the suitable resistant material such as polyethylene, polyvinyl chloride, and polyvinyl esters, capable of withstanding the chemical action of these solutions are available. Also filter screens and heat exchange equipment to withstand the chemical action of these solutions are available. Therefore it is possible to maintain close solution control necessary for continuous operation.

Examples of other ways and means for chemically milling metals are herewith presented. A metal may be removed by spraying the solution onto it so as to have a fine stream of the reactant solution contact the metal. By this technique deep grooving can be realized by rotating a part. In another manner a pipe may be made lighter-in-weight by running the solution through it so as to de-

crease the wall thickness. As is realized the interior wall of the pipe is eaten away and the inside diameter thereby enlarged.

From the above description of our discovery it is seen that the same is applicable to the chemical milling of metals and alloys. From our discovery it is possible to save considerable waste in the manufacture of metal products; to produce the parts in batches or continuously; the capital investment for production of the components may be as low as approximately 5 to 10 percent of the capital investment for equivalent machine milling. Also, it is possible to produce highly complex shapes and configurations with chemical milling which are not possible with machine milling, to use non-symmetrical patterns with chemical milling which are difficult to use with machine milling, to produce integrally stiffened structures whereby one unit serves as a structure instead of an integrally fabricated structure depending upon welds, which are weaker than the metal itself, to produce a structure, and to make tapered structural materials which are difficult to make with machine milling. Furthermore, from an engineering design standpoint it is seen that it is possible to etch after forming the structure. In many operations it is economically feasible to obtain closer tolerances, to have a number of various steps to cut, and to mill all surfaces of the part simultaneously. In this regard, it is possible to chemically mill with equal ease all types of martensitic steel. From a labor standpoint and skilled artisan viewpoint it is not necessary in chemical milling to use as highly skilled operators as in machine milling.

Having described our discovery, what we claim and wish to protect is as follows:

1. An aqueous acidic composition of matter adapted for chemically milling metal which contains chloride, nitrate and a ferric ion therein, the chloride concentration being at least about 1.0 normal, the nitrate concentration being at least about 0.75 normal, the ferric concentration being at least about .07 molar, the available hydrogen ion concentration being however, at least 1.8 normal, said composition further including a minor amount of a member selected from the group consisting of ammonium chloride and stannic chloride, ammonium chlorostannate and mixture thereof.
2. The composition of claim 1 containing also a weak acid having a primary ionization constant in the range of  $10^{-4}$  to  $10^{-6}$ .
3. An aqueous acidic composition of matter adapted for chemically milling metal and which contains a chloride, a nitrate and a ferric ion therein, the chloride concentration computed as 38% HCl being at least about 9% by weight, the nitrate concentration computed as 70% nitric acid being at least about 5%, the ferric concentration computed as ferric chloride being at least about 1%, all percentages being by weight, the available hydrogen ion concentration being, however, at least 1.8 normal, said composition further including a minor amount of a member selected from the group consisting of ammonium chloride and stannic chloride, ammonium chlorostannate and mixtures thereof.
4. An aqueous acidic composition of matter adapted for chemically milling metal which contains a chloride, a nitrate and a ferric ion therein, the chloride concentration computed as 38% HCl being in the range of about 9-25%, the nitrate concentration computed as 70% nitric acid being in the range of about 5-25%, the ferric concentration computed as ferric chloride being about 1-26%, all percentages being by weight, said composition further including a minor amount of a member selected from the group consisting of ammonium chloride and stannic chloride, ammonium chlorostannate and mixtures thereof.
5. The composition of claim 4 containing also from about 1-6% of a weak acid having a primary ionization constant in the range of  $10^{-4}$  to  $10^{-6}$ .

6. A process for manufacturing a metal structure from steel, said process including covering portions of the steel with a protective covering, subjecting the uncovered steel to the action of an aqueous acidic composition of matter adapted for chemically milling metal which contains a chloride, a nitrate and a ferric ion therein, the chloride concentration being at least about 1.0 normal, the nitrate concentration being at least about 0.75 normal, the ferric concentration being at least about .07 molar, the available hydrogen ion concentration being, however, at least 1.8 normal, said composition further including a minor amount of a member selected from the group consisting of ammonium chloride and stannic chloride, ammonium chlorostannate, and mixtures thereof.

7. A process for manufacturing a metal structure from steel, said process including covering portions of the steel with a protective covering, subjecting the uncovered steel to the action of an aqueous acidic composition of matter adapted for chemically milling metal, which contains a chloride, a nitrate and ferric ion therein, the chloride concentration computed as 38% HCl being at least about 9% by weight, the nitrate concentration computed as 70% nitric acid being at least about 5%, the ferric concentration computed as ferric chloride being at least about 1%, the available hydrogen ion concentration being, however, at least 1.8 normal, said composition further including a minor amount of a member selected from the group consisting of ammonium chloride and stannic chloride, ammonium chlorostannate and mixtures thereof.

8. A process for manufacturing a metal structure from martensitic steel, said process including covering portions of the raw material metal with a protective covering and subjecting the uncovered raw material metal to the action of an aqueous acidic composition of matter adapted for chemically milling metal, which contains chloride, nitrate and ferric moieties therein, the chloride concentration computed as 38% HCl being in the range of about 9-25%, the nitrate concentration computed as 70% nitric acid being in the range of about 5-25%, the ferric concentration computed as ferric chloride being about 1-25%, said composition further including a minor amount of a member selected from the group consisting of ammonium chloride and stannic chloride, ammonium chlorostannate and mixtures thereof, and from about 1-6% of a weak acid having a primary ionization constant in the range of  $10^{-4}$  to  $10^{-6}$ , all percentages being by weight.

20 References Cited in the file of this patent

UNITED STATES PATENTS

|           |            |       |               |
|-----------|------------|-------|---------------|
| 469,704   | Knidermann | ----- | Mar. 1, 1892  |
| 2,429,107 | Petren     | ----- | Oct. 14, 1947 |
| 2,446,060 | Pray       | ----- | July 27, 1948 |

25 OTHER REFERENCES

Thum: Book of Stainless Steel, 2nd ed., Amer. Soc. of Metals, Cleveland, Ohio, © Jan. 1935, p. 151.

30 Monypenny: V. 2., 3rd ed., rev. 1954, Chapman & Hall, London, p. 253.